# EUROPEAN PATENT APPLICATION

(11) **EP 4 050 139 A1**
(43) Date of publication of application: **31.08.2022**
(21) Application number: 21382155.6
(22) Date of filing: 24.02.2021
(51) Int. Cl.: D03D 15/25, D02G 3/12, D03D 15/217, D03D 15/283, D02G 3/44, D02G 3/04

(54) **ANTIBACTERIAL AND BREATHABLE COTTON POLYESTER TEXTILE**

(71) Applicant: Ramon Castillo, Miguel, 08026 BARCELONA (ES)
(72) Inventor: Ramon Castillo, Miguel, 08026 BARCELONA (ES)
(74) Representative: Isern Patentes y Marcas S.L.

(57) **Abstract**

The present invention is related to a fabric having antibacterial properties, among other, comprising cotton and polyester fibre yarns, wherein the polyester fibre yarn comprises copper filaments and to the process thereof. Additionally, the invention relates to the use of said textile in the manufacturing of protective clothing for health personnel, hygienic footwear covers, protective face mask, table clothing for hotels and/or restaurants or systems to purify air, such as air condition systems. Furthermore, the invention relates to a process to manufacture said textile.

## Description

### Field of the invention

The present invention is related to a fabric having antibacterial properties, among other, comprising cotton and polyester fibre yarns, wherein the polyester fibre yarn comprises oxidized copper filaments and to the process thereof. Furthermore, the invention relates to the use of said textile in the manufacturing of protective clothing for health personnel, hygienic footwear covers, protective face mask, table clothing for hotels and/or restaurants or in systems to purify air, such as air condition systems.

### State of the art

In recent years, society has experienced quick change in their habits towards preventing health infections as well as reducing their transmission rates, more particularly with the last worldwide deceases such as SARS-CoV-1 or MERS or the worldwide pandemic caused by SARS-CoV-2

In this sense, in the field of antibacterial textiles, needs to be developed fast to be able to meet the actual demand to manufacture and deliver different products which have antibacterial properties and can filter dangerous pathogens.

The areas where exists more demand in today's society, are those areas related to health facilities as well as public places, where health personnel as well as civilian personnel need to be able to perform the work duties as well as reduce the infection transmission rate when using public facilities such as public transport or offices. Therefore, clothing, face masks or public fair filtering systems have become essential alternative elements for the prevention or reduction of the transmission rate of different infection which may occur in the work place, public places as well as in health centres.

Hence, there is the need to provide textil material which can be effective against different pathogens, such as virus and/or bacteria, as well as being, strong, flexible, breathable and reusable.

### Brief description

The present invention solves the problems described in the state of the art, since it provides a textile, as described in the first aspect of the invention, which has good antibacterial properties, so is effective against different pathogens, such as, small particles and aerosols as well as virus and/or bacteria. Furthermore, the textile is breathable and reusable, as can be sterilised by a wide range of sterilisation techniques without effecting the properties of the textile.

The first aspect of the invention relates to a fabric with antibacterial properties comprising cotton fibre yarns and polyester fibre yarns, characterized in that:
- The cotton fibre yarns are present in a weight percentage from 70% up to 90% to the total weight of the fabric and the weight to the polyester fibres from are present in a weight percentage from 10% up to 30% and
- The polyester fibbers yarns comprise copper filaments, wherein the copper filaments are present in a range from 2 and 0.05 % by weight to the weight of the polyester fibre yarn.

The second aspect of the invention relates to a process to produce the fabric according to first aspect the process comprising at least the following steps:
- providing a blend comprising cotton fibre yarns and polyester-copper composite fibre yarns, wherein the cotton fibre yarns are present in the blend in an amount from 70-90 % and the polyester-copper composite fibre yarns in an amount of 10-30 %;
- intertwining the at least one or more than one cotton fibre yarns and one or more polyester-copper composite fibre yarns in the multi-filament's fibre yarns tightly and closely to provide a composite line which contains from 70-90 % of cotton fibre yarns and from 10-30 % of polyester-copper composite fibre yarns;
- interweaving multiple composite lines longitudinally and latitudinally to construct a fabric having an antibacterial-properties.

The third aspect of the invention relates to the use of the fabric of the first aspect as a filter material or barrier against viruses selected from the list consisting of coronavirus, rotaviruses, retroviruses, type IV viruses and polioviruses. Preferably wherein the virus is selected from the list consisting of VHB, VHC y el VIH, orthomyxoviridae, Mers-cov, Ebola virus and SARS-CoV-2 virus. Preferably, as a filter material or barrier used in protective clothing for health personnel, hygienic footwear covers, in a protective face mask, table clothing for hotels and/or restaurants or in systems to purify air, preferably air condition systems

The forth aspect relates to protective clothing for healthcare personnel comprising the fabric according to the first aspect of the invention. Preferably the protective clothing for healthcare personnel, is selected from the list consisting of, lab coats, shirts, t-shirts, trousers, hygienic footwear covers, and face masks.

The fifth aspect relates to bags for containing and/or transferring contaminated sanitary clothing to laundry facilities comprising a fabric according to the first aspect.

### Detailed description

The first aspect of the invention relates to a fabric with antibacterial properties comprising cotton fibre yarns and polyester fibre yarns, characterized in that:
- The cotton fibre yarns are present in a weight percentage from 70% up to 90% to the total weight of the fabric and the weight to the polyester fibres from are present in a weight percentage from 10% up to 30% and
- The polyester fibbers yarns comprise copper filaments, wherein the copper filaments are present in a range from 2 and 0.05 % by weight to the weight of the polyester fibre yarn and wherein the copper filaments are oxidized copper filaments.

The presence of copper oxides on the surface of nanoparticles is not highly desirable in many industries. Surprisingly, it has been observed that the fabric of the invention has very good antibacterial properties when the copper filaments included in the polyester fibers are oxidized. This characteristic provides the textile with very good antibacterial properties against bacteria and viruses. Therefore, oxidized copper particles comprise a layer of cuprous oxide (Cu₂O) on their surface. The content of cuprous oxide in the copper filament may range from 20% to 80% by weight, this provides very good antibacterial properties against bacteria and viruses.

In a preferred embodiment of the fabric of the first aspect, the copper filaments are present in a range from 2 to 0.2% by weight to the weight of the polyester, more preferably from 1 to 0.3 %. When the amount of copper filaments is below 0.05 % the fabric of the first aspect is not show antibacterial properties.

In a preferred embodiment of the fabric of the first aspect, the ooxidized copper filaments comprise a layer of cuprous oxide on its surface, preferably, the content of the cuprous oxide in the filament is in a range from 20% hasta el 80% by weight of the filament.

In a preferred embodiment of the fabric of the first aspect, the polyester is a textured polyester yarn.

In another preferred embodiment of the fabric of the first aspect, the cotton fibre yarns are present in a ratio by weight to the polyester fibres yarn from 90:10 to 70:30, preferably, from 87:13 to 75:25 %.

For the sake of clarity, the term the polyester fibres comprising oxidised copper filaments are also referred as to polyester-copper composite fibre, likewise polyester fibre yarns comprising oxidised copper filaments are also referred as polyester-copper composite fibre yarns.

The term antibacterial encompasses, being suited and effective to prevent the growth of bacteria and viruses and/or being able to act as a barrier and a filter against aerosols, particles and/or bacteria.

In another preferred embodiment of the fabric of the first aspect, the cotton fibre yarns and the polyester fibre yarns are intertwined forming composite lines and wherein the diameter of the intertwined composite lines is in a range from 250 to 80 µm, preferably from 180 to 110 µm, providing a strong textile suitable to be used as protective clothing for hotels and/or restaurants, face masks, protective clothing for health facilities and centres.

In another preferred embodiment of the fabric of the first aspect, the polyester-copper composite fibre yarn has a coefficient of variation of tenacity, CV _{τ} (a) %, from 4-2.5 and /or an elongation, CV %, from 10-30 from 10-30%, preferably the elongation, CV %, may be from 10-24%, these characteristics provide the fabric of the first aspect with suitable strength and suitable flexibility for the intended uses.

In another preferred embodiment of the fabric of the first aspect, the fabric has a grammage from 150-300 g/m₂, preferably from 200-280 g/m₂. So, the fabric of the first aspect shows good mechanical and breathable properties.

In another preferred embodiment of the fabric of the first aspect, the warp of the fabric is from 25-10 threads/cm, preferably from 20 hasta 14 threads/cm y/o la the weft is from 5-15, preferably from 8 to 12 threads/cm. So, the fabric is strong and breathable

The fabric according to any of the preceding claims, has a boiling water shrinkage % from 4-1%, preferably from 3,5 to 1 %, therefore the fabric is suitable for being washed many times and for being reusable. The shrinkage test in boiling water was performed on a Texturmat-Me tester according to DIN 53866-12.

The fabric of the first aspect presents the advantages that is breathable and has high level of water absorption and prevent condensation, which is a very good property when used as a protective face mark. It also retains its properties after washing, even if washed at high temperature, which makes is suitable to be used several times, as a protective face mark or as air conditioning filter respectively.

Preferably the fabric of the first aspect does not comprise latex and/or natural rubbers.

The fabric of the first aspect can be further processed by sewing and is also printable

The fabric was successfully tested for different uses, such as protective face mask, hygienic footwear covers, protective clothing for health centres and facilities, table clothing for hotels and/or restaurants or air conditioning filters in systems to purify air, such as air condition systems

The second aspect of the invention relates to a process to produce the fabric according to first aspect the process comprising at least the following steps:
(a) providing a blend comprising cotton fibre yarns and polyester-copper composite fibre yarns, wherein the cotton fibre yarns are present in the blend in an amount from 70-90 % and the polyester-copper composite fibre yarns in an amount of 10-30 %;
(b) intertwining the at least one or more than one cotton fibre yarns and one or more polyester-copper composite fibre yarns in the multi-filament's fibre yarns tightly and closely to provide a composite line which contains from 70-90 % of cotton fibre yarns and from 10-30 % of polyester-copper composite fibre yarns;
(c) interweaving multiple composite lines longitudinally and latitudinally to construct a fabric having an antibacterial-properties.

The process to prepare the polyester fibre yarns comprising cupper filaments of the first aspect, also referred as polyester-copper composite fibre yarns, is carried out by means of melting extrusion process, the process comprises at least the steps of:
- Provide a mixture of the polyester material and the copper filaments, preferably wherein the polyester material is in the form of pellets, granulate or chips;
- Provide the mixture obtain in the previous step in a melting furnace, preferably the melting furnaces is an extruder, at a temperature from 10-240 °C, preferably from 190 to 230 °C;
- Kneading the resulting polyester-copper filaments composite mixture at a temperature from 180 to 240 °C, preferably by means of an extruder nozzle, to provide polyester-copper filaments composite fibres;
- Drawing the polyester-copper filaments composite fibres obtained in the previous step to provide the polyester-copper filaments composite fibre yarns;
- preferably by grouping them together and twisting them to provide the polyester-copper filaments composite fibre yarns;
- Optionally, allowing the polyester-copper filaments composite fibre yarns to drop thir temperature to below 40 °C and rolling of the resulting solidified polyester-copper filaments composite fibre yarns in a bobbin.

The third aspect of the invention relates to the use of the fabric of the first aspect as a filter material or barrier against viruses selected from the list consisting of coronavirus, rotaviruses, retroviruses, type IV viruses and polioviruses. Preferably wherein the virus is selected from the list consisting of VHB, VHC y el VIH, orthomyxoviridae, Mers-cov, Ebola virus and SARS-CoV-2 virus and/or against aerosols and/or against particles. Preferably, as a filter material or barrier used in protective clothing suitable for health personnel, hygienic footwear covers, in a protective face mask, table clothing for hotels and/or restaurants or in systems to purify air, preferably air condition systems

The forth aspect relates to protective clothing for healthcare personnel comprising the fabric according to the first aspect of the invention. Preferably the protective clothing for healthcare personnel, is selected from the list consisting of, lab coats, shirts, t-shirts, trousers, hygienic footwear covers, and face masks.

The fifth aspect relates to bags for containing and/or transferring contaminated sanitary clothing to laundry facilities comprising a fabric according to claims 1-9.

Filter for air-conditioning systems comprising the fabric according to claims 1-9.

### Examples and experimental teste results

The textile comprising cotton fibre yarns and polyester fibre yarns, characterized in that the cotton fibre yarns are present in a weight percentage of 88% to the total weight of the fabric and the weight to the polyester fibres are 12 % to the total weight of the fabric, wherein the polyester fibres yarns comprise oxidized copper filaments in an amount of 0.6% by weight to the weight of the polyester fibre yarns and wherein oxidized copper filaments comprised a layer of cuprous oxide on its surface. The fabric was prepared following the process described in the present application.

The fabric was tested for its suitability to filtration based on the standards described in UNE-EN 13274, for respiratory equipment

Aerosol tests have been performed on monodisperse and polydisperse systems characterized by a sufficient concentration of particles of (3 + 0.5) microns.
Aerosol filtration efficacy: >96%.
Particle filtration efficacy: >93%.
Good efficacy against bacteria filtration, complying with all standards of UNE-EN14683:2019+AC2019, for face mask equipment.

The test results demonstrated that the fabric was a good as a barrier and good filtering material against corona virus, covid-19. The tests also shown that the textile prevented moisture condensation, thus was very suitable to be used as a protective face mask

The antimicrobial and antivirus efficacy were demonstrated when the tests IS015020743 and IO 15018184 were performed. The textile also meets all criteria established by EU BPR y EU REACH.

It was demonstrated that the fabric can be sterilised in an ozone sterilisation chamber, and said process did not altered the characteristics of the textile.

The fabric was also be sterilized by means of autoclave at 121°C.

Furthermore, the textile was disinfected by means of UV light, said sterilisation means being effective to sterilised the fabric against, the coronavirus SARS- CoV o MERSCoV (1, 15-18). Also, it was tested complying with the tests described in UNE-EN149, against the coronavirus, SARS- CoV-2 and MERSCoV (1, 15-18) and shown that particles with a diameter of 0.3 microns and grater that 0.3 microns were filtered with an efficacy of at least 96%.

## Claims

1. A fabric with antibacterial properties comprising cotton fibre yarns and polyester fibre yarns, **characterized in that**:
- The cotton fibre yarns are present in a weight percentage from 70% up to 90% to the total weight of the fabric and the weight to the polyester fibres from are present in a weight percentage from 10% up to 30% and
- The polyester fibbers yarns comprise copper filaments, wherein the copper filaments are present in a range from 2 and 0.05 % by weight to the weight of the polyester fibre yarn and wherein the copper filaments are oxidized copper filaments.

2. The fabric according to the preceding claims, wherein the copper filaments are present in a range from 2 to 0.2% by weight to the weight of the polyester, more preferably from 1 to 0.3 %.

3. The fabric according to any of the preceding claims, wherein oxidized copper filaments comprise a layer of cuprous oxide on its surface and optionally wherein the content of the cuprous oxide in the filament is in a range from 20% to 80% by weight.

4. The fabric according to any of the preceding claims, wherein the polyester is a textured polyester yarn.

5. The fabric according to any of the preceding claims, wherein the cotton fibre yarns and the polyester fibre yarns are intertwined forming composite lines and wherein the diameter of the intertwined composite lines is in a range from 250 to 80 µm, preferably from 180 to 110 µm.

6. The fabric according to any of the preceding claims, has a boiling water shrinkage % from 4-1%.

7. The fabric according to any of the preceding claims, wherein the polyester fibre yarns has a coefficient of variation of tenacity from entre 4-2.5 and /or an elongation from 10-30 %.

8. The fabric according to any of the preceding claims, where the fabric has a grammage from 150-300 g/m₂, preferably from 200-280 g/m₂

9. The fabric according to any of the preceding claims, wherein the warp is from 25-10 threads/cm, preferably from 20 hasta 14 threads/cm y/o la the weft is from 5-15, preferably from 8 to 12 threads/cm

10. Process to produce the fabric according to claims 1-10 comprising at least the following steps:
(a) providing a blend comprising cotton fibre yarns and polyester-copper composite fibre yarns, wherein the cotton fibre yarns are present in the blend in an amount from 70-90 % and the polyester-copper composite fibre yarns in an amount of 10-30 %;
(b) intertwining the at least one or more than one cotton fibre yarns and one or more polyester-copper composite fibre yarns in the multi-filament's fibre yarns tightly and closely to provide a composite line which contains from 70-90 % of cotton fibre yarns and from 10-30 % of polyester-copper composite fibre yarns;
(c) interweaving multiple composite lines longitudinally and latitudinally to construct a fabric having an antibacterial-properties

11. Use of the fabric according to any of the preceding claims 1-9 as a filter material against particles, aerosols, bacteria and viruses selected from the list consisting of coronavirus, rotaviruses, retroviruses, type IV viruses and polioviruses, preferably wherein the virus is selected from the list consisting of VHB, VHC y el VIH, orthomyxoviridae, Mers-cov, Ebola virus and SARS-CoV-2 virus.

12. Use of the fabric according to the preceding claim, as a filter material and/or a barrier in protective clothing for health personnel, hygienic footwear covers, protective face mask or in systems to purify air.

13. Protective clothing for healthcare personnel comprising the fabric according to claims 1-9, preferably wherein the protective clothing for healthcare personnel, is selected from the list consisting of, lab coats, shirts, t-shirts, trousers, hygienic footwear covers, and face masks.

14. Bags for containing or/and transferring contaminated sanitary clothing to laundry facilities, comprising a fabric according to claims 1-9.

15. Filter for air-conditioning systems comprising the fabric according to claims 1-9.
